



US005419951A

United States Patent [19]

Golz

[11] Patent Number: 5,419,951

[45] Date of Patent: May 30, 1995

[54] CUT AND ABRASION RESISTANT  
WEBBING AND MULTIFILAMENT  
BICOMPONENT YARN USED IN THE  
MANUFACTURING THEREOF

[75] Inventor: Robert E. Golz, Swansea, Mass.

[73] Assignee: Murdock Webbing Company, Inc.,  
Central Falls, R.I.

[21] Appl. No.: 71,536

[22] Filed: Jun. 4, 1993

#### Related U.S. Application Data

[63] Continuation-in-part of Ser. No. 687,836, Apr. 19,  
1991, Pat. No. 5,219,636.

[51] Int. Cl.<sup>6</sup> ..... B32B 23/02; D04H 1/04;  
D02G 3/00; B66C 1/12

[52] U.S. Cl. ..... 428/229; 428/245;  
428/259; 428/296; 428/373; 139/411; 294/74

[58] Field of Search ..... 428/193, 245, 259, 296,  
428/373, 229; 139/411; 294/74

#### [56] References Cited

##### U.S. PATENT DOCUMENTS

|           |         |                     |         |
|-----------|---------|---------------------|---------|
| 3,526,565 | 9/1970  | Walter .....        | 428/193 |
| 3,629,053 | 12/1971 | Kimura et al. ....  | 428/374 |
| 4,052,095 | 10/1977 | Johnson .....       | 428/172 |
| 4,856,837 | 8/1989  | Hammersla, Jr. .... | 294/74  |
| 4,987,030 | 1/1991  | Saito et al. ....   | 428/373 |
| 5,167,263 | 12/1992 | Kelen et al. ....   | 139/383 |
| 5,219,636 | 6/1993  | Golz .....          | 428/193 |

Primary Examiner—George F. Lesmes

Assistant Examiner—Terrel Morris

Attorney, Agent, or Firm—Salter & Michaelson

#### [57] ABSTRACT

Sling or tie-down webbing in the form of a strap provided with protective warp yarn structure made up of bicomponent fibers that include a polyester core with a sheath of a polymer with a lower melting point than the polyester, which webbing has been subjected to a heat treatment sufficient to cause melting of said sheath, but not of the core.

6 Claims, 3 Drawing Sheets









FIG. 6



FIG. 7

**CUT AND ABRASION RESISTANT WEBBING AND  
MULTIFILAMENT BICOMPONENT YARN USED  
IN THE MANUFACTURING THEREOF**

**BACKGROUND OF THE INVENTION**

This application is a continuation-in-part of applicant's U.S. application Ser. No. 07/687,836, filed Apr. 19, 1991 and entitled CUT AND ABRASION RESISTANT WEBBING, scheduled to issue on Jun. 15, 1993 under U.S. Pat. No. 5,219,636.

In the movement of heavy materials, it is common practice to use a crane or hoist whose downwardly-extending cable is provided with a hook, the hook being connected to the load by one or more flexible slings. A sling of this type usually consists of an elongated webbing having a soft eye at each end for engagement with the horn of the hook. The bight of the sling passes under the load and transfers the weight from the load to the hook.

Because the load is often a massive article with sharp edges, such as steel I-beams and the like, the sling can be and frequently is subjected to an abrasive action. When excessive wear takes place, it is usually at the edge of the sling and this can lead to breakage of the sling. Because the material being lifted is not only heavy but also awkward in shape, the possibility of accidental breakage of the supporting sling cannot be tolerated. The appearance of the slightest wear on the sling leads, therefore, to its being discarded, which is an expensive action. In addition, separation or weakening of the sling can take place even before visible wear takes place, because it is sometimes loaded to over its safe working load.

In addition, webbing of the type above described is often used to tie down heavy cargo, where it is desired to secure the cargo against movement. Such tie-down webbing is also subjected to abrasion and cutting at its edges, and hence the same problems that exist with cargo slings also exist with tie-down webbing.

Because wear, i.e., abrasion or cutting, seems to take place most readily on the edges of the webbing, attempts have been made in the past to increase the resistance to wear at that part of the sling. Various methods for increasing the wear and cut resistance of the edges of fabric strips have been developed, as shown in the Johnson U.S. Pat. No. 2,659,958 (Fourdrinier wire having reinforced coated marginal portions), in the Walter U.S. Pat. No. 3,526,565 (treated warp yarn made into sheet, then heated to fuse and form a web), in the Miller U.S. Pat. No. 3,571,814 (bead of plastic material along the strip), in the Dominick U.S. Pat. No. 3,632,383 (application of a heat-solidifiable composition to the edge), and in the Weatherly et al U.S. Pat. No. 4,501,782 (bonding webs by use of ultrasonic energy). The Johnson U.S. Pat. No. 4,052,095 shows a sling whose surface is protected by a lamina of an elastomeric material. The Ayase U.S. Pat. No. 4,600,626 shows an automobile seat belt whose resistance to lateral flexure is increased by the use of stiff weft yarns. The Hammersla U.S. Pat. No. 4,856,837 shows a cargo sling that is provided with protective warp yarns consisting of a vinyl sheath on a polyester core. Unfortunately, none of these prior art structures, with the possible exception of Hammersla, gives adequate protection against abrasion to the edge of the strip where it is needed. The degree of resistance to cutting and abrasion is determined in those structures

by the material from which the protective yarns are made.

Whereas applicant's aforementioned copending application is concerned with and covers protection of the edges of the webbing against abrasion or cutting, it has been found that in certain situations, such as, for example, in lumber sorting slings used for the lifting and transporting of logs, the face of the sling or webbing comes in contact with the load and hence requires added protection against abrasion and cutting.

Thus, it is a primary object of the present invention to provide a woven sling or webbing having extraordinary resistance to abrasion and cutting throughout its surface.

More specifically, it is an object of this invention to provide a sling or webbing having specially formed protective yarns that extend in the warp direction intermediate the edges of the webbing so as to impart resistance to abrasion or cutting throughout the face of the webbing.

It is a further object to provide such a webbing with the specially formed yarns extending longitudinally as stripes.

It is a still further object to provide such a webbing with the specially formed yarns extending longitudinally across the full face of the webbing.

Another object is the provision of such a webbing with the specially formed warp yarns located on both the face and the back of the webbing.

With these and other objects in view, as will be apparent to those skilled in the art, the invention resides in the combination of parts set forth in the specification and covered by the claims appended hereto.

**SUMMARY OF THE INVENTION**

In general, the present invention has to do with a sling which has an elongated main body made up of warp yarns of a synthetic fiber, which body is covered with a ply using woven polymer yarns having longitudinal warp yarns and lateral weft yarns. Specially formed protective warp yarns are arranged intermediate the edges of the main body, said yarns being formed of multiple filaments which each have a core and an outer sheath, with the latter melting at a temperature lower than the core. Specifically, the bicomponent filament has a polyester core which melts at around 489 degrees F. and has a sheath selected from a group consisting of nylon-6, polypropylene, or polyethylene, or any other fiber having a lower melting point.

In carrying out the objectives of my invention, the webbing with its protective yarns is subjected to a temperature treatment that is sufficient to melt the sheath component, but not the core, the result being that the fused sheaths integrate and impart improved resistance to cutting and abrasion. The bicomponent fiber has substantially the same modulus of elasticity as the synthetic fiber in the main body so as not to inhibit elongation of the strap. After the temperature treatment, the webbing may be subjected to a cracking operation to increase its flexibility, while not decreasing its resistance to wear.

**BRIEF DESCRIPTION OF THE DRAWINGS**

The character of the invention, however, may be best understood by reference to one of its structural forms, as illustrated by the accompanying drawings, in which:

FIG. 1 is a perspective view of a lumber sorting sling constructed in accordance with the principles of the

present invention, and shown in use in lifting a load of logs;

FIG. 2 is a perspective view, somewhat enlarged, of the invention, showing its general structure;

FIG. 3 is a transverse sectional view of the sling, taken on the line 3—3 of FIG. 2, showing the protective warp yarns on one face of the sling in the form of stripes;

FIG. 4 is a view similar to FIG. 3 but showing the protective yarns extending across one face of the sling;

FIG. 5 is a view similar to FIG. 3 but showing the protective stripes on both the face and back of the sling;

FIG. 6 is a fragmentary plan view of the sling showing the protective stripes located intermediate the edges thereof; and

FIG. 7 is a cross-sectional view, on an enlarged scale, of the bicomponent yarn that forms a critical part of the invention.

#### DESCRIPTION OF THE PREFERRED EMBODIMENT

Referring first to FIG. 1, which best shows the general features of the invention, the sling, indicated generally by the reference numeral 10, is shown in use to hold a load of logs 12. The sling extends upwardly from the load to hoisting hooks 14.

In FIG. 2, it can be seen that the sling 10 is an elongated strap with eyes formed at opposite ends. The eyes are formed by folding the strap back on itself and stitching the free end to the bight of the strap, as at 15.

In FIG. 3, it can be seen that the sling 10 is provided with a main body 16 made up of warp yarns 18 formed of any suitable fiber and packed to form a rectangular cross-section having narrow end edges 20, 22 (see FIG. 2). The main body is surrounded by an outer ply 24 consisting of woven yarns 26. The ply is formed with longitudinal warp yarns 28 and transverse or lateral weft yarns 30. Specially formed protective warp yarns 32 are arranged so as to extend longitudinally intermediate the edges 20, 22 of the main body. Each protective yarn (FIG. 7) consists of bicomponent multiple filaments 38, each having a core and an outer sheath, the latter having a lower melting temperature than the core.

Specifically, each protective yarn consists of bicomponent multiple filaments 38 which have a polyester core 34 which melts at a temperature of around 489 degrees F. and a sheath 36 that is formed of a polymer selected from the group consisting of nylon-6, polypropylene, or polyethylene, or any other fiber having a lower melting point than the core.

In FIGS. 3 and 6, the protective warp yarns 32 are provided at three locations along the face of the sling 10 so as to in effect form stripes thereon. In FIG. 4 the protective yarns extend across the entire face of the sling, while in FIG. 5 the protective yarns are in the form of stripes on both the face and back of the sling. Although not specifically shown, the protective yarns 32 in FIG. 4 could also cover both the entire face and the entire back of the sling.

Once the sling has been constructed in the manner described above, it is subjected to a temperature treatment that is sufficient to melt the sheath 36, but not the core 34. As a result of this melting or fusing operation, the molecular characteristics of yarn 32, and particularly sheath 36, are somewhat altered, resulting in an unexpectedly high resistance to abrasion. In addition, the melting operation results in some degree of fusion between the filaments of each yarn as well as fusion

between adjacent protective yarns 32, resulting in a web-like structure that further enhances resistance to abrasion and cutting.

In a preferred version of the invention, the bicomponent fiber has a sheath of nylon-6 that is treated for 4 minutes at about 435 degrees F. Another version of the invention uses a sheath of polypropylene that is treated for 4 minutes at around 375 degrees F. A still further version of the invention uses a sheath of polyethylene which is treated for 4 minutes at a temperature of around 300 degrees F. In all cases, the bicomponent fiber has substantially the same modulus of elasticity as the synthetic fiber of the yarns 18 of the main body, even after the fusing operation. It may be desirable, although not essential, to subject the sling, after the temperature treatment, to a cracking operation to increase its flexibility, while not decreasing its resistance to abrasion and to cutting. In all of the above cases, the degree of heat is sufficient to melt or fuse the sheath 36, but not core 34.

The operation and advantages of the invention will now be readily understood in view of the above description. When the sling 10 is used in the manner shown in FIG. 1, it is clear that certain types of loads 12 cause extreme wear to the surfaces of the sling. In the present case, as the hoist hook rises and the forces between the sling and the load take place, the reinforcing and protective yarns 32 that extend longitudinally along the sling can receive the stresses without being cut or even abraded. The tough nature of the structure formed by these yarns serves to completely protect the sling from such damaging treatment.

It can be seen, then, that the present invention has the advantage that the location of the special bicomponent fibers (that have been exposed to temperature treatment) protect the most vulnerable portion of the sling, i.e., those portions that are in contact with a load having rough surfaces, such as logs. Additionally, this protection can be provided inexpensively during the manufacture of the webbing.

It is obvious that minor changes may be made in the form and construction of the invention without departing from the material spirit thereof. It is not, however, desired to confine the invention to the exact form herein shown and described, but it is desired to include all such as properly come within the scope claimed.

The invention having been thus described, what is claimed as new and desired to secure by Letters Patent is:

50. What is claimed is:

1. An elongated webbing formed from warp and weft yarns woven together, said webbing comprising face and back surfaces, at least some of said warp yarns being specially formed so as to exhibit increased resistance to abrasion and cutting, said specially formed warp yarns each comprising a plurality of individual filaments each of which comprises a core and an outer sheath, the melting point of the sheath being lower than that of its core, said specially formed yarns being located intermediate the longitudinal edges of said webbing, said webbing having been subjected to a heat treatment sufficient to melt said sheaths, but not said cores, said specially formed yarns, after heat treatment, having at least as great a modulus of elasticity as the yarns in said webbing that have not been specially formed.

2. The webbing as recited in claim 1 wherein said filaments each have a polyester core which melts at around 489 degrees F. and a sheath selected from the

group consisting of nylon-6, polypropylene, and poly-ethylene.

3. The webbing of claim 2 wherein said specially formed yarns comprise a plurality of longitudinally extending stripes.

4. The webbing of claim 3 wherein said stripes are located on the face surface of said webbing.

5. The webbing of claim 3 wherein said stripes are located on the back surface of said webbing.

6. The webbing of claim 1 wherein said specially formed yarns extend across the full width of said webbing.

\* \* \* \* \*

10

15

20

25

30

35

40

45

50

55

60

65